

Patented Apr. 10, 1923.

1,451,125

UNITED STATES PATENT OFFICE.

BERTRAND S. SUMMERS, OF PORT HURON, MICHIGAN.

PROCESS FOR THE PRODUCTION OF PAPER PULP AND THE LIKE.

No Drawing.

Application filed April 21, 1922. Serial No. 555,898.

To all whom it may concern:

Be it known that I, BERTRAND S. SUMMERS, a citizen of the United States, residing at Port Huron, county of Saint Clair, and 5 State of Michigan, have invented certain new and useful Improvements in Processes for the Production of Paper Pulp and the like, of which the following is a specification.

10 My invention relates more particularly to what is known as the sulfite process for the digestion of wood to reduce it to the state of pulp, though the invention is not limited to the treatment of wood. In this process as 15 commonly practiced the wood, after having been stripped of the bark is reduced to chips of suitable size and cooked in a solution of what is known as bisulfite of calcium, though the material may contain more or less mag- 20 nesium or indeed other bi-sulfites may be employed. While this material is commonly known as bi-sulfite, it does not strictly conform to formula and where I have used the term I wish it to be understood as signify- 25 ing an acid salt of sulfurous acid or a sulfite dissolved in sulfurous acid. For the purpose of my invention the bi-sulfite may be made up in any usual or approved manner and used in the usual proportions to the 30 material to be treated, though my invention is not limited thereto.

My invention is based upon the discovery that if a proper amount of a reducing agent is introduced into the cooking acid (the bi- 35 sulfite solution) considerably enhanced yields of pulp are obtained and the product is of a better quality. I have found that the best results are obtained by introducing into the cooking acid a relatively small 40 amount of hydro-sulfurous acid. Hydro- sulfurous acid is a powerful reducing agent, which, under proper conditions is converted by oxidation into sulfurous acid, without undue precipitation of sulfur. When this 45 material is added to or produced in the liquor in which the pulp is digested the proper reducing conditions occur to produce the increased and improved yield referred to above. It is to be understood that where I 50 use the term hydro-sulfurous acid herein- after I include therein salts of the acid and also materials which are capable of produc- 55 ing the acid when added to the digesting liquor. I may mention as a suitable source of hydro-sulfurous acid, sodium hydro-sulfite, which is an article of com-

merce and may be obtained upon the market. When an acid such as sulfurous acid is added to this salt free hydro-sulfurous acid is formed. Thus when the salt is added 60 to the cook in the process of digesting wood the sulfurous acid in the liquor reacts with the salt producing hydro-sulfurous acid and sodium sulfite, according to the equation



The hydro-sulfurous acid gradually combines with the calcium sulfite present during the progress of the digestion, the reaction being somewhat obscure but in all probability, a calcium hydro-sulfite is formed according to the equation



The presence of the calcium sulfite in the 75 cooking liquor seems to have a pronounced influence in preserving the hydro-sulfurous acid from decomposition, except in the manner above noted, and the hydro-sulfurous acid in some manner affects the action of the 80 calcium sulfite to increase the yield and quality of the pulp, apparently by preventing the liquor from attacking the cellulose.

While my process may be performed as above described, by the addition of sodium 85 hydro-sulfite to the liquor, I prefer to form the hydro-sulfurous acid in the liquor by the addition of a suitable metal such as zinc or magnesium. When zinc is dissolved in 90 sulfurous acid hydro-sulfurous acid is generated according to the following equation



Therefore when zinc or other suitable metal is added to the cook in the sulfite process it reacts with the sulfurous acid present, forming hydro-sulfurous acid. Preferably the zinc is added in the form of a powder and it is convenient to sprinkle it on the chips as they are charged into the digester. If some metal other than zinc is used the proper quantity may be determined from the ratio of its atomic weight to that of zinc. As sodium hydro-sulfite is very soluble it may be added to the acid before it is introduced into the digester. For practical purposes a pound of zinc may be taken as the equivalent of a pound of the sodium hydro-sulfite.

The quantity of sodium hydro-sulfite or powdered zinc to be used varies considerably in accordance with the result desired. Ordinarily ten to twenty pounds thereof

may be used in a 10 ton digester holding about 22,000 gallons of liquor and about 30 tons of chips, the strength of the acid being about 4 per cent, of which approximately 5 2.60 per cent is free acid and 1.40 per cent combined. With such a charge I have found twelve pounds of zinc dust to be a very satisfactory addition. If the metal or 10 sodium hydro-sulfite addition is increased beyond the proportions mentioned the pulp begins to get too tough to work well in the machinery utilized in reducing it, though for certain purposes where a tougher pulp is 15 required the proportions of zinc or sodium hydro-sulfite may be somewhat greater than that mentioned.

From the above it will be evident that my process may be practical without altering the conditions of paper pulp manufacture 20 or the apparatus used except by the addition of the material for furnishing hydro-sulfurous acid and this is true as well of the so-called quick-cook or Ritter-Kelner process as of the Mitscherlich or slow-cook 25 process.

I claim:

1. A process of producing sulfite wood

pulp, which consists in cooking the wood in a solution containing a bi-sulfite and hydro-sulfurous acid.

2. A process of producing sulfite wood pulp, which consists in cooking the wood in a solution containing a bi-sulfite and a material capable of producing hydro-sulfurous acid.

3. A process of producing sulfite wood pulp, consisting in cooking the wood in a solution of bi-sulfite containing a metal capable of producing with the bi-sulfite hydro-sulfurous acid.

4. A process for producing sulfite wood pulp, which consists in cooking the wood in a solution containing bi-sulfite and a compound of hydro-sulfurous acid.

5. A process of preparing sulfite wood pulp, which consists in cooking the wood in a solution containing bi-sulfite in the presence of zinc.

6. The herein described process of preparing vegetable fibres consisting in cooking the same in a solution containing a bi-sulfite and hydro-sulfurous acid.

BERTRAND S. SUMMERS.